

## UNITED STATES PATENT OFFICE

KURT SPONSEL, OF FRANKFORT-ON-THE-MAIN-HOCHST, AND KURT JOCHUM, OF FRANKFORT-ON-THE-MAIN, GERMANY, ASSIGNORS TO I. G. FARBBENINDUSTRIE AKTIENGESELLSCHAFT, OF FRANKFORT-ON-THE-MAIN, GERMANY, A CORPORATION OF GERMANY

PROCESS OF STRENGTHENING COTTON, ARTIFICIAL SILK, ARTIFICIAL FOILS OF CELLULOSE, VISCOSE, OR THE LIKE AND MATERIAL PREPARED BY THIS PROCESS

No Drawing. Application filed August 2, 1929, Serial No. 383,152, and in Germany August 10, 1928.

The present invention relates to threads, whereas the parent material has only a breaking strength of 174 g. and an elongation of 6%.  
The present invention relates to threads, fabrics and sheets of cellulose, such as, for example, cotton or artificial silk, containing glyoxal residues.

5 We have found that threads, fabrics and sheets of cellulose, such as, for example, cotton or artificial silk, containing glyoxal residues highly surpass the parent materials in regard to breaking strength, elongation and the 10 manner in which the interstices are closed. Such articles of manufacture can be prepared by treating hanks of cotton or artificial silk or sheets of viscose with glyoxal or an agent splitting off glyoxal, for instance, in a dilute 15 aqueous solution, subsequently squeezing off the excess and gently drying the material.

The material can also be impregnated in vacuo. This aftertreatment has the advantage over the known treatment with form- 20 aldehyde that no pressure apparatus is required, that the temperature need not be raised and that the workmen are not injured by the odorless glyoxal.

The above-mentioned improvement in the 25 properties of the said cellulose materials by the treatment with glyoxal or an agent splitting off glyoxal is due to a chemical reaction. During the impregnation, the glyoxal combines with the hydroxy groups of the cellulose materials thereby forming acetal-like 30 products which have the desired properties.

The following examples illustrate the invention, but are not intended to limit it there- 35 to:

(1) Viscose artificial silk, after being precipitated, is treated in a bath containing 2 g. of glyoxal, 3 g. of sodium dimethyl-aniline-p-sulfonate and 10. g. of glycerine per liter, freed from the excess of liquid by squeezing 40 it through rubber rollers and dried. The strength of the product thus obtained has increased 50% whereas the elongation of 7% has remained unaltered.

(2) Ammoniacal copper oxide silk is im- 45 pregnated with a solution of glyoxal of 2% strength at a temperature of 20° C., squeezed through rubber rollers and dried at a temperature of between 50° C. and 60° C. The product thus obtained has a breaking 50 strength of 213 g., an elongation of 9.3%,

We claim:  
1. As new articles of manufacture threads, 55 fabrics and sheets of cellulose containing glyoxal residues.  
2. Artificial silk of viscose containing glyoxal residues.  
3. Cuprammonium silk containing gly- 60 oxal residues.

In testimony whereof, we affix our signatures.

KURT SPONSEL.

KURT JOCHUM.

65

70

75

80

85

90

95

100